

## UNITED STATES PATENT OFFICE

2,304,025

PROCESS FOR COLOR DEVELOPMENT OF  
PHOTOGRAPHIC MATERIALS

Wilhelm Schneider, Dessau in Anhalt, and Gustav Wilmanns, Wolfen, Kreis Bitterfeld, Germany, assignors to General Aniline & Film Corporation, New York, N. Y., a corporation of Delaware

No Drawing. Application February 28, 1940, Serial No. 321,209. In Germany February 23, 1939

3 Claims. (Cl. 95—88)

This invention relates to color photography and more particularly to color development of photographic materials.

It has been proposed to use in the production of photographic color pictures as developing agent for color development of silver halide emulsions, developers as such phenylene diamine, aminophenol, dihydroxybenzene.

Phenylene diamines, amino phenols and dihydroxybenzenes are frequently used as developing agents in known processes for color development of silver halide emulsion layers. These developing agents together with suitable color formers, for instance phenols, anilines and compounds with reactive methylene and methyl groups, form quinone imine- and azomethine dyes, depending on the color formers used, by means of the exposed silver salt. After dissolving the silver formed during the reaction, a pure dyestuff image is obtained. The color formers or the developing agents or both may be added to the developing solution or incorporated into the emulsion layers.

Images of sufficient color density and brilliancy are obtained in the process of modern color development, after correct developing to  $\gamma$ -infinity. They show, however, a too contrasty gradation. For a medium gradation with harmonious tone values required in most cases, development to  $\gamma$ -infinity is not desirable. However, in such a case the sensitivity of the material is only partly utilised and there is the disadvantage, that the colors become very thin and pervious to a large amount of white light during the copying process, which results in blackish copies.

It is an object of the present invention to provide a process for color development of photographic materials.

A further object resides in the provision of an improved color-developer containing novel components for color development of a harmonious, not too contrasty gradation.

Still further objects will become apparent from the detailed specification following hereinafter.

This invention is based on the observation, that color images of excellent brilliancy and not too contrasty are obtained, when heterocyclic nitrogen-containing bases are added to the color-developer.

Suitable heterocyclic bases are for instance piperidine, piperazine, lysidine.

Especially effective developers are obtained according to the new process.

It was already known to add diamines to 55

reversal-developers for black and white development, but from the effect of these developers nobody could predict the results obtained by the new process.

5 The process is applicable to color development with developers containing the color formers in the solution and to color development of silver halide emulsions containing the color formers in the emulsion layer itself. When using silver halide emulsion layers with color formers contained therein, color formers fast to diffusion according to the following U. S. Patents are especially suitable: 2,178,612, 2,179,-234, 2,179,238, and 2,179,239, issued on November 7, 1939; and 2,186,849, issued on January 9, 1940.

In the following examples such developers are described:

## Example I

|                                              |       |     |
|----------------------------------------------|-------|-----|
| Water                                        | liter | 1   |
| Diethyl-p-phenylene-diamine chlorine hydrate | grams | 2.5 |
| Sodium sulfite                               | do    | 0.5 |
| Potassium bromide                            | do    | 2.5 |
| Potassium carbonate                          | do    | 75  |
| Piperidine                                   | do    | 0.9 |

## Example II

|                                              |       |     |
|----------------------------------------------|-------|-----|
| Water                                        | liter | 1   |
| Diethyl-p-phenylene-diamine chlorine hydrate | grams | 2.5 |
| Potassium carbonate                          | do    | 75  |
| Sodium sulfite                               | do    | 0.5 |
| Potassium bromide                            | do    | 2.5 |
| Pyrrolidine                                  | do    | 0.5 |

Time for development 10 minutes.

## Example III

|                                              |       |     |
|----------------------------------------------|-------|-----|
| Water                                        | liter | 1   |
| Diethyl-p-phenylene-diamine chlorine hydrate | grams | 2.5 |
| Potassium carbonate                          | do    | 75  |
| Sodium sulfite                               | do    | 0.5 |
| Potassium bromide                            | do    | 2.5 |
| Morpholine                                   | do    | 4   |

Time for development 10 minutes.

What we claim is:

1. A color forming photographic developer comprising a primary aromatic amino developing agent, a compound which couples with the oxidation product of the developing agent on photographic development to produce a dyestuff and a nitrogen-containing heterocyclic base selected from the group consisting of piperidine, pyrrolidine, morpholine, piperazine and lysidine.

2. A color forming photographic developer consisting of a p-phenylene diamine salt as a primary aromatic amino developing agent, a compound which couples with the oxidation product of the developing agent on photographic development to produce a dyestuff and a nitrogen-containing heterocyclic base, selected from the group consisting of piperidine, pyrrolidine, morpholine, piperazine and lysidine.

3. A color forming photographic developer 10

consisting of diethyl p-phenylene diamine salt as a primary aromatic amino developing agent, a compound which couples with the oxidation product of the developing agent on photographic development to produce a dyestuff and a nitrogen-containing heterocyclic base selected from the group consisting of piperidine, pyrrolidine, morpholine, piperazine and lysidine.

WILHELM SCHNEIDER.  
GUSTAV WILMANNS.